

H. JOHNSON.

PACKING RESIN AS AN ARTICLE OF COMMERCE.

No. 184,969.

Patented Dec. 5, 1876.



WITNESSES

*W. T. Johnson.*  
*Edmund Gruborito.*

*Hardy Johnson*  
INVENTOR

# UNITED STATES PATENT OFFICE.

HARDING JOHNSON, OF WILMINGTON, NORTH CAROLINA.

## IMPROVEMENT IN PACKING ROSIN AS AN ARTICLE OF COMMERCE.

Specification forming part of Letters Patent No. **184,969**, dated December 5, 1876; application filed November 17, 1876.

*To all whom it may concern:*

Be it known that I, HARDING JOHNSON, of the city of Wilmington and State of North Carolina, have invented a new and useful Improvement in the Packing of Rosin as an Article of Commerce, which improvement is fully set forth in the following specification.

The object of my invention is to afford a package of rosin convenient for either the retail or wholesale dealer in the article, so as to enable them to avoid the trouble, and attendant great inconveniences, in dealing out the article to their customers, such as the soiling of clothes, injury to goods, &c., caused by rosin dust.

My invention consists of rosin melted and shaped in molds and packages, rosin reduced to powder and packed, or rosin cut into regular shapes and packages.

I claim as my invention—

As an improved article of merchandise, rosin either melted and molded into shape, cut into blocks, or powdered and packed, as described.

HARDING JOHNSON.

Witnesses:

W. T. JOHNSON,  
EDMUND SZUBORITS.